



US008088234B2

(12) **United States Patent**  
**Khosla et al.**

(10) **Patent No.:** **US 8,088,234 B2**  
(b5) **Date of Patent:** **Jan. 3, 2012**

(54) **AA2000-SERIES ALUMINUM ALLOY PRODUCTS AND A METHOD OF MANUFACTURING THEREOF**

(75) Inventors: **Sunil Khosla**, Beverwijk (NL); **Andrew Norman**, Beverwijk (NL); **Hugo Van Schooneveldt**, Noordbeemster (NL)

(73) Assignee: **Aleris Aluminum Koblenz GmbH**, Koblenz (DE)

(\*) Notice: Subject to any disclaimer, the term of this patent is extended or adjusted under 35 U.S.C. 154(b) by 116 days.

(21) Appl. No.: **11/773,900**

(22) Filed: **Jul. 5, 2007**

(65) **Prior Publication Data**

US 2008/0210349 A1 Sep. 4, 2008

**Related U.S. Application Data**

(60) Provisional application No. 60/818,965, filed on Jul. 7, 2006.

(51) **Int. Cl.**

*C22F 1/04* (2006.01)  
*C22C 21/06* (2006.01)  
*C22C 21/16* (2006.01)  
*C22C 21/12* (2006.01)  
*C22C 21/08* (2006.01)  
*C22C 21/04* (2006.01)

(52) **U.S. Cl. ....** **148/552; 148/439; 148/440; 420/529; 420/534; 420/535; 420/537; 420/546**

(58) **Field of Classification Search ....** **148/437-440, 148/522, 552; 420/528, 529, 531-535, 537, 420/542-547**

See application file for complete search history.

(56) **References Cited**

U.S. PATENT DOCUMENTS

2,249,349 A 7/1941 Deutsch  
3,287,185 A 11/1966 Vachet  
3,305,410 A 2/1967 Sublett et al.  
3,418,090 A 12/1968 Fritzlen  
3,674,448 A 7/1972 Brown et al.  
3,791,876 A 2/1974 Kroger  
3,791,880 A 2/1974 Hunsicker et al.  
3,794,531 A 2/1974 Markworth  
3,826,688 A 7/1974 Levy  
3,857,973 A 12/1974 McKee et al.  
3,881,966 A 5/1975 Staley et al.  
3,984,259 A 10/1976 Rogers, Jr. et al.  
4,140,549 A 2/1979 Chia et al.  
4,189,334 A 2/1980 Dubost et al.  
4,196,021 A 4/1980 Bouvaist et al.  
4,305,763 A 12/1981 Quist et al.  
4,462,843 A 7/1984 Baba et al.  
4,462,893 A 7/1984 Moriya et al.  
4,477,292 A 10/1984 Brown  
4,589,932 A 5/1986 Park  
4,618,382 A 10/1986 Miyagi et al.  
4,659,393 A 4/1987 Bouvaist et al.  
4,711,762 A 12/1987 Vernam et al.  
4,713,216 A 12/1987 Higashi et al.

4,828,631 A 5/1989 Ponchel et al.  
4,927,470 A 5/1990 Cho  
4,946,517 A 8/1990 Cho  
4,954,188 A 9/1990 Ponchel et al.  
4,976,790 A 12/1990 McAuliffe et al.  
4,988,394 A 1/1991 Cho  
5,108,520 A 4/1992 Liu et al.  
5,186,235 A 2/1993 Word, Jr.  
5,213,639 A 5/1993 Colvin et al.  
5,221,377 A 6/1993 Hunt, Jr. et al.  
5,277,719 A 1/1994 Kuhlman et al.  
5,312,498 A 5/1994 Anderson  
5,313,639 A 5/1994 Chao  
5,356,495 A 10/1994 Wyatt-Mair et al.  
5,496,423 A 3/1996 Wyatt-Mair et al.  
5,496,426 A 3/1996 Murtha  
5,560,789 A 10/1996 Sainfort et al.  
5,593,516 A 1/1997 Cassada, III  
5,624,632 A 4/1997 Baumann et al.  
5,681,405 A 10/1997 Newton et al.  
5,718,780 A 2/1998 Bryant et al.  
5,738,735 A 4/1998 Bechet  
5,833,775 A 11/1998 Newton et al.  
5,858,134 A 1/1999 Bechet et al.  
5,865,911 A 2/1999 Miyasato et al.  
5,865,914 A 2/1999 Karabin et al.  
5,888,320 A 3/1999 Dorward  
5,938,867 A 8/1999 Dorward et al.  
6,027,582 A 2/2000 Shahani et al.  
6,120,623 A 9/2000 Gupta et al.  
6,129,792 A 10/2000 Murtha  
6,224,992 B1 5/2001 Delbeke et al.  
6,238,495 B1 5/2001 Haszler  
6,315,842 B1 11/2001 Shahani et al.  
6,337,147 B1 1/2002 Haszler et al.  
6,444,058 B1 9/2002 Liu et al.  
6,543,122 B1 4/2003 Perkins et al.  
6,562,154 B1 5/2003 Rioja et al.  
6,569,542 B2 5/2003 Warner et al.

(Continued)

FOREIGN PATENT DOCUMENTS

DE 68927149 6/1987

(Continued)

OTHER PUBLICATIONS

U.S. Appl. No. 11/773,919, Khosla et al., filed Jul. 5, 2007.

(Continued)

*Primary Examiner* — Roy King

*Assistant Examiner* — Caitlin Kiechle

(74) *Attorney, Agent, or Firm* — Novak Druce + Quigg, LLP

(57) **ABSTRACT**

An AA2000-series alloy including 2 to 5.5% Cu, 0.5 to 2% Mg, at most 1% Mn, Fe <0.25%, Si >0.10 to 0.35%, and a method of manufacturing these aluminum alloy products. More particularly, disclosed are aluminum wrought products in relatively thick gauges, i.e. about 30 to 300 mm thick. While typically practiced on rolled plate product forms, this method may also find use with manufacturing extrusions or forged product shapes. Representative structural component parts made from the alloy product include integral spar members, and the like, which are machined from thick wrought sections, including rolled plate.

## U.S. PATENT DOCUMENTS

|              |    |         |                    |    |            |         |
|--------------|----|---------|--------------------|----|------------|---------|
| 6,602,361    | B2 | 8/2003  | Warner et al.      | FR | 2716896    | 9/1995  |
| 6,627,330    | B1 | 9/2003  | Shimizu et al.     | FR | 2841263    | 12/2003 |
| 6,652,678    | B1 | 11/2003 | Marshall et al.    | FR | 2846669    | 5/2004  |
| 6,726,878    | B1 | 4/2004  | Fridlyander et al. | GB | 2855834    | 12/2004 |
| 6,743,308    | B2 | 6/2004  | Tanaka et al.      | GB | 925956 B   | 5/1963  |
| 6,790,407    | B2 | 9/2004  | Fridlyander        | GB | 0952288    | 3/1964  |
| 6,972,110    | B2 | 12/2005 | Chakrabarti et al. | GB | 1029486    | 5/1966  |
| 6,994,760    | B2 | 2/2006  | Benedictus et al.  | GB | 1231090    | 5/1971  |
| 7,060,139    | B2 | 6/2006  | Senkovet et al.    | GB | 1273261    | 5/1972  |
| 7,097,719    | B2 | 8/2006  | Bray et al.        | GB | 1427657    | 3/1976  |
| 7,250,223    | B2 | 7/2007  | Miyachi et al.     | GB | 2065516    | 7/1981  |
| 7,294,213    | B2 | 11/2007 | Warner et al.      | GB | 1603690    | 11/1981 |
| 7,550,110    | B2 | 6/2009  | Warner et al.      | GB | 2114601    | 8/1983  |
| 7,666,267    | B2 | 2/2010  | Benedictus et al.  | JP | 2430937    | 4/2007  |
| 2001/0006082 | A1 | 7/2001  | Warner et al.      | JP | 59126762   | 7/1984  |
| 2001/0039982 | A1 | 11/2001 | Sigli et al.       | JP | 61049796   | 3/1986  |
| 2002/0011289 | A1 | 1/2002  | Warner             | JP | 62010246   | 1/1987  |
| 2002/0014288 | A1 | 2/2002  | Warner et al.      | JP | 62122744   | 6/1987  |
| 2002/0014290 | A1 | 2/2002  | Dif et al.         | JP | 62122745   | 6/1987  |
| 2002/0039664 | A1 | 4/2002  | Magnusen et al.    | JP | 63319143   | 6/1987  |
| 2002/0121319 | A1 | 9/2002  | Chakrabarti et al. | JP | 1039340    | 2/1989  |
| 2002/0150498 | A1 | 10/2002 | Chakrabarti et al. | JP | 1208438    | 8/1989  |
| 2002/0153072 | A1 | 10/2002 | Tanaka et al.      | JP | 2047244    | 2/1990  |
| 2002/0162609 | A1 | 11/2002 | Warner             | JP | 06128678   | 5/1994  |
| 2003/0140990 | A1 | 7/2003  | Ribes et al.       | JP | 6228691    | 8/1994  |
| 2003/0219353 | A1 | 11/2003 | Warner et al.      | JP | 8120385    | 5/1996  |
| 2004/0007295 | A1 | 1/2004  | Lorentzen et al.   | JP | 8144031    | 6/1996  |
| 2004/0101434 | A1 | 5/2004  | Fridlyander et al. | JP | 09-279284  | 10/1997 |
| 2004/0109787 | A1 | 6/2004  | Haszler et al.     | JP | 10280081   | 10/1998 |
| 2004/0211498 | A1 | 10/2004 | Keidel et al.      | JP | 10298692   | 11/1998 |
| 2005/0006010 | A1 | 1/2005  | Benedictus et al.  | JP | 2001020028 | 1/2001  |
| 2005/0034794 | A1 | 2/2005  | Benedictus et al.  | JP | 2001115227 | 4/2001  |
| 2005/0067066 | A1 | 3/2005  | Tanaka et al.      | JP | 2002241882 | 8/2002  |
| 2005/0072497 | A1 | 4/2005  | Eberl et al.       | RU | 2003147498 | 5/2003  |
| 2005/0081965 | A1 | 4/2005  | Benedictus et al.  | RU | 2044098    | 9/1995  |
| 2005/0095447 | A1 | 5/2005  | Baumann et al.     | RU | 1625043    | 10/1995 |
| 2005/0189044 | A1 | 9/2005  | Benedictus et al.  | RU | 2165996    | 4/2001  |
| 2006/0016523 | A1 | 1/2006  | Dif et al.         | RU | 2184166 C2 | 6/2002  |
| 2006/0032560 | A1 | 2/2006  | Benedictus et al.  | RU | 2215058    | 10/2003 |
| 2006/0174980 | A1 | 8/2006  | Benedictus et al.  | RU | 2215807 C2 | 11/2003 |
| 2006/0182650 | A1 | 8/2006  | Eberl et al.       | RU | 2215808    | 11/2003 |
| 2007/0000583 | A1 | 1/2007  | Rioja et al.       | RU | 2003106552 | 10/2004 |
| 2007/0151636 | A1 | 7/2007  | Buerger et al.     | SU | 664570     | 5/1979  |
| 2007/0204937 | A1 | 9/2007  | Buerger et al.     | WO | 9203586    | 3/1992  |
| 2008/0173377 | A1 | 7/2008  | Khosla et al.      | WO | 9526420    | 10/1995 |
| 2008/0173378 | A1 | 7/2008  | Khosla et al.      | WO | 9610099    | 4/1996  |
| 2009/0269608 | A1 | 10/2009 | Benedictus et al.  | WO | 9628582    | 9/1996  |
| 2009/0320969 | A1 | 12/2009 | Benedictus et al.  | WO | 9629440    | 9/1996  |

## FOREIGN PATENT DOCUMENTS

|    |              |         |  |    |                |         |
|----|--------------|---------|--|----|----------------|---------|
| DE | 102004010700 | 10/2004 |  | WO | 9837251        | 8/1998  |
| DE | 10392805     | 6/2005  |  | WO | 0054967        | 9/2000  |
| EP | 0081441      | 6/1983  |  | WO | 0210468        | 2/2002  |
| EP | 0368005      | 5/1990  |  | WO | 02052053       | 7/2002  |
| EP | 0587274      | 3/1994  |  | WO | 02075010       | 9/2002  |
| EP | 0605947      | 7/1994  |  | WO | 03076677       | 9/2003  |
| EP | 0670377      | 9/1995  |  | WO | 04001080       | 12/2003 |
| EP | 0377779      | 10/1997 |  | WO | 2004044256     | 5/2004  |
| EP | 0799900      | 10/1997 |  | WO | 2004/090183 A1 | 10/2004 |
| EP | 0829552      | 3/1998  |  | WO | 2004111282     | 12/2004 |
| EP | 0876514      | 11/1998 |  | WO | 2005003398     | 1/2005  |
| EP | 989195       | 3/2000  |  | WO |                |         |
| EP | 1026270      | 8/2000  |  | WO |                |         |
| EP | 1045043      | 10/2000 |  | WO |                |         |
| EP | 1114877      | 7/2001  |  | WO |                |         |
| EP | 1143027      | 10/2001 |  | WO |                |         |
| EP | 1158068      | 11/2001 |  | WO |                |         |
| EP | 1170394      | 1/2002  |  | WO |                |         |
| EP | 1231290      | 8/2002  |  | WO |                |         |
| EP | 1306455      | 5/2003  |  | WO |                |         |
| EP | 1382698 A1   | 1/2004  |  | WO |                |         |
| FR | 1508123      | 1/1968  |  | WO |                |         |
| FR | 2066696      | 8/1971  |  | WO |                |         |
| FR | 2163281 A5   | 7/1973  |  | WO |                |         |
| FR | 2234375      | 1/1975  |  | WO |                |         |
| FR | 2409319      | 6/1979  |  | WO |                |         |
| FR | 2472618      | 7/1981  |  | WO |                |         |

## OTHER PUBLICATIONS

- U.S. Appl. No. 11/773,904, Khosla et al., filed Jul. 5, 2007.  
 Airbus Industrie Material Specification AIMS 03-02-020 (Feb. 2002).  
 Hufnagel, W., Key to Aluminium Alloys, 4th Edition, Aluminium-Schlüssel = Key to Aluminium Alloys, pp. 195-205 (XP-002194851) (1991).  
 International Preliminary Report on Patentability in application PCT/EP2007/005972 mailed on Jan. 22, 2009, international stage of U.S. Appl. No. 11/773,900, (11 pages).  
 International Preliminary Report on Patentability in application PCT/EP2007/005973 mailed on Jan. 22, 2009, international stage of U.S. Appl. No. 11/773,904 (12 pages).  
 International Preliminary Report on Patentability in application PCT/EP2007/005975 mailed on Jan. 22, 2009, international stage of U.S. Appl. No. 11/773,919, (12 pages).

- Office action for U.S. Appl. No. 11/480,558, mailed Dec. 31, 2008 (14 pages).
- Vojtech et al., Improving the casting properties of high-strength aluminum alloys. *Materiali in Technologiji* 38 (2004), pp. 99-102.
- Office action for U.S. Appl. No. 11/773,904, mailed Mar. 16, 2009 (18 pages).
- Office action for U.S. Appl. No. 11/773,919, mailed Mar. 16, 2009 (21 pages).
- P.T. Houldcroft, "A Simple Cracking Test for Use with Argon-Arc Welding", *British Welding Journal*, Oct. 1955, pp. 471-475.
- Pechiney Aluminium: "Demi produits aluminium; Caractéristiques générales—Aluminium mill products; general properties;" Oct. 1985, *Announcement Pechiney Aluminium*, pp. 1-5, XP002240985.
- M.S. degree thesis of L.E. Oswald, titled "Effects of microstructure on high-cycle fatigue of an Al—Zn—Mg—Cu alloy (AL-7055)", pp. i-x and 1-54 (Apr. 2003).
- Office action of Jul. 15, 2009 from U.S. Appl. No. 11/480,558.
- Office action of Sep. 9, 2009 from U.S. Appl. No. 11/566,630.
- Office action of Sep. 29, 2009 from U.S. Appl. No. 11/773,904.
- Office action of Sep. 25, 2009 from U.S. Appl. No. 11/773,919.
- Advisory action of Oct. 30, 2009 from U.S. Appl. No. 11/480,558.
- The conversion table for hardness and tensile strength value—DIN EN ISO 18265—Nov. 2003.
- Arai et al., *ASM Handbook, Heat Treating of Aluminum Alloys—Strengthening by Heat Treatment*, ASM International, vol. 4, 1995, p. 5-7.
- Final Rejection dated Mar. 11, 2010, in co-pending U.S. Appl. No. 11/566,630.
- Final Rejection dated Mar. 4, 2010, in co-pending U.S. Appl. No. 11/773,904.
- "Heat Treating of Aluminum Alloys," *ASM Handbook*, vol. 4, pp. 841-856, 1995.
- Lakhtin Yu. M. et al. *Material Science*, Moscow, "Machine Construction" 1980, p. 40.
- V.I. Dobatkin, *Smelting and Casting of Aluminum Alloys*, Moscow, "Metallurgy", 1970, p. 27.
- The Russian State Standard GOST 4784-97; Aluminum and wrought aluminum alloys, rades, Minsk, Publisher of Standards, 1999, p. 7, 8, Table 6.
- International Alloy Designations and Chemical Composition Limits for Wrought Aluminum and Wrought Aluminum Alloys (teak sheets). The Aluminum Association, miscellaneous annotated pages (Jul. 1998).
- "Aluminum Viewed from Within", Altenpohl, 1st edition, pp. 118-131 (1982).
- ASM Specialty Handbook, Aluminum and Aluminum Alloys, edited by J.R. Davis, ASM International, pp. 247-248, 1993.
- Aluminum Properties and Physical Metallurgy, edited by J.E. Hatch, American Society for Metals, p. 112-113 (1984).
- Aluminium-Taschenbuch 15. Auflage, Dorosel et al., p. 20-25 (1999).
- Advisory Action mailed in U.S. Appl. No. 11/773,919 on Dec. 15, 2009, 3 pages.
- Non-Final Rejection mailed in U.S. Appl. No. 11/773,919 on Jun. 8, 2010, 14 pages.
- Advisory Action mailed in U.S. Appl. No. 11/566,630 on Jun. 24, 2010, 3 pages.
- Final Rejection mailed in U.S. Appl. No. 11/566,630 on Mar. 11, 2010, 10 pages.
- Requirement for Restriction / Election mailed in U.S. Appl. No. 11/566,630 on Jun. 19, 2009, 6 pages.
- Final Rejection mailed in U.S. Appl. No. 12/547,466 on Jul. 12, 2010, 13 pages.
- Non-Final Rejection mailed in U.S. Appl. No. 12/547,466 on Jan. 28, 2010, 11 pages.
- Advisory Action mailed in U.S. Appl. No. 10/819,130 on May 6, 2008, 4 pages.
- Advisory Action mailed in U.S. Appl. No. 10/819,130 on Jul. 13, 2009, 3 pages.
- Final Rejection mailed in U.S. Appl. No. 10/819,130 on Jan. 25, 2008, 9 pages.
- Final Rejection mailed in U.S. Appl. No. 10/819,130 on Feb. 26, 2009, 7 pages.
- Non-Final Rejection mailed in U.S. Appl. No. 10/819,130 on Jun. 22, 2007, 8 pages.
- Non-Final Rejection mailed in U.S. Appl. No. 10/819,130 on Aug. 5, 2008, 8 pages.
- Requirement for Restriction / Election mailed in U.S. Appl. No. 10/819,130 on Apr. 3, 2007, 5 pages.
- Advisory Action mailed in U.S. Appl. No. 10/821,184 on Jun. 4, 2008, 4 pages.
- Final Rejection mailed in U.S. Appl. No. 10/821,184 on Nov. 21, 2008, 9 pages.
- Final Rejection mailed in U.S. Appl. No. 10/821,184 on Feb. 21, 2008, 14 pages.
- Non-Final Rejection mailed in U.S. Appl. No. 10/821,184 on Jun. 26, 2007, 11 pages.
- Non-Final Rejection mailed in U.S. Appl. No. 10/821,184 on Sep. 3, 2008, 14 pages.
- Requirement for Restriction / Election mailed in U.S. Appl. No. 10/821,184 on Apr. 3, 2007, 5 pages.
- Advisory Action mailed in U.S. Appl. No. 10/976,154 on Nov. 21, 2008, 4 pages.
- Final Rejection mailed in U.S. Appl. No. 10/976,154 on Oct. 15, 2009, 17 pages.
- Final Rejection mailed in U.S. Appl. No. 10/976,154 on May 29, 2008, 18 pages.
- Non-Final Rejection mailed in U.S. Appl. No. 10/976,154 on Feb. 18, 2009, 16 pages.
- Non-Final Rejection mailed in U.S. Appl. No. 10/976,154 on Sep. 20, 2007, 15 pages.
- Advisory Action mailed in U.S. Appl. No. 11/239,651 on Feb. 24, 2009, 3 pages.
- Advisory Action mailed in U.S. Appl. No. 11/239,651 on Mar. 23, 2010, 3 pages.
- Final Rejection mailed in U.S. Appl. No. 11/239,651 on Oct. 14, 2008, 10 pages.
- Final Rejection mailed in U.S. Appl. No. 11/239,651 on Dec. 7, 2009, 10 pages.
- Non-Final Rejection mailed in U.S. Appl. No. 11/239,651 on Feb. 22, 2008, 13 pages.
- Non-Final Rejection mailed in U.S. Appl. No. 11/239,651 on Jun. 1, 2009, 10 pages.
- Non-Final Rejection mailed in U.S. Appl. No. 11/239,651 on Jun. 8, 2010, 20 pages.
- Non-Final Rejection mailed in U.S. Appl. No. 12/497,987 on May 26, 2010, 10 pages.
- Advisory Action mailed in U.S. Appl. No. 11/773,904 on Jun. 11, 2010, 3 pages.
- Final Rejection mailed in U.S. Appl. No. 11/773,904 on Mar. 4, 2010, 23 pages.
- U.S. Appl. No. 11/733,919—Final Office action mailed Nov. 18, 2010.
- ASM Specialty Handbook Aluminum and Aluminum Alloys, J.R. Davis, ASM International, pp. 290-295 and 319-320 (1993).
- Kuhlman, *Forging of Aluminum Alloys—Forging Methods*, vol. 14A, ASM Handbook, ASM International, p. 1-6 (2005).
- U.S. Appl. No. 11/773,904—Non-Final Office action mailed Dec. 22, 2010.
- U.S. Appl. No. 11/566,630—Non-Final Office action mailed Nov. 29, 2010.
- U.S. Appl. No. 12/497,987—Final Office action mailed Jan. 6, 2011.
- U.S. Appl. No. 11/239,651—Notice of Allowance mailed Sep. 24, 2010.
- U.S. Appl. No. 12/547,466—Non-Final Office action mailed Mar. 31, 2011.
- U.S. Appl. No. 11/566,630—Final Office action mailed Apr. 5, 2011.
- U.S. Appl. No. 11/773,919—Advisory Office action mailed Mar. 7, 2011.
- Final Office Action mailed Sep. 7, 2011 in U.S. Appl. No. 12/547,466 (15 pages).
- Non-Final Office Action mailed Aug. 12, 2011 in U.S. Appl. No. 12/497,987 (9 pages).

## 1

**AA2000-SERIES ALUMINUM ALLOY  
PRODUCTS AND A METHOD OF  
MANUFACTURING THEREOF**

**CROSS REFERENCE TO RELATED  
APPLICATION**

This claims the benefit of U.S. provisional application No. 60/818,965, filed Jul. 7, 2006, incorporated herein by reference.

**FIELD OF THE INVENTION**

This invention relates to an AA2000-series alloy comprising 2 to 5.5% Cu, 0.5 to 2% Mg, at most 1% Mn, Fe <0.25%, Si >0.10 to 0.35%, and to a method of manufacturing these aluminum alloy products. More particularly, the invention relates to aluminum wrought products in relatively thick gauges, i.e. about 30 to 300 mm thick. While typically practiced on rolled plate product forms, this invention may also find use with manufacturing extrusions or forged product shapes. Representative structural component parts made from the alloy product include integral spar members and the like which are machined from thick wrought sections, including rolled plate. This invention is particularly suitable for manufacturing high strength extrusions and forged aircraft components. Such aircraft include commercial passenger jetliners, cargo planes and certain military planes. In addition, non-aerospace parts like various thick mould plates or tooling plates may be made according to this invention.

**BACKGROUND TO THE INVENTION**

As will be appreciated herein below, except as otherwise indicated, alloy designations and temper designations refer to the Aluminum Association designations in Aluminum Standards and Data and the Registration Records, as published by the Aluminum Association in 2006.

For any description of alloy compositions or preferred alloy compositions, all references to percentages are by weight percent unless otherwise indicated.

Different types of aluminum alloys have been used in the past for forming a variety of products for structural applications in the aerospace industry. Designers and manufacturers in the aerospace industry are constantly trying to improve fuel efficiency, product performance and constantly trying to reduce the manufacturing and service costs. The preferred method for achieving the improvements, together with the cost reduction, is the uni-alloy concept, i.e. one aluminum alloy that is capable of having improved property balance in the relevant product forms.

State of the art at this moment is high damage tolerant AA2x24 (i.e. AA2524) or AA6x13 or AA7x75 for fuselage sheet, AA2324 or AA7x75 for lower wing, AA7055 or AA7449 for upper wing and AA7050 or AA7010 or AA7040 or AA7140 for wing spars and ribs or other sections machined from thick plate. The main reason for using different alloys for each different application is the difference in the property balance for optimum performance of the whole structural part.

For fuselage skin, damage tolerant properties under tensile loading are considered to be very important, that is a combination of fatigue crack growth rate ("FCGR"), plane stress fracture toughness and corrosion. Based on these property requirements, high damage tolerant AA2x24-T351 (see e.g. U.S. Pat. No. 5,213,639 or EP-1026270-A1) or Cu containing AA6xxx-T6 (see e.g. U.S. Pat. No. 4,589,932, U.S. Pat. No.

## 2

5,888,320, US-2002/0039664-A1 or EP-1143027-A1) would be the preferred choice of civilian aircraft manufacturers.

For lower wing skin a similar property balance is desired, but some toughness is allowably sacrificed for higher tensile strength. For this reason AA2x24 in the T39 or a T8x temper are considered to be logical choices (see e.g. U.S. Pat. No. 5,865,914, U.S. Pat. No. 5,593,516 or EP-1114877-A1).

For upper wing, where compressive loading is more important than the tensile loading, the compressive strength, fatigue (SN-fatigue or life-time or FCGR) and fracture toughness are the most critical properties. Currently, the preferred choice would be AA7150, AA7055, AA7449 or AA7x75 (see e.g. U.S. Pat. No. 5,221,377, U.S. Pat. No. 5,865,911, U.S. Pat. No. 5,560,789 or U.S. Pat. No. 5,312,498). These alloys have high compressive yield strength with at the moment acceptable corrosion resistance and fracture toughness, although aircraft designers would welcome improvements on these property combinations.

10 For thick sections having a thickness of more than 3 inch or parts machined from such thick sections, a uniform and reliable property balance through thickness is important. Currently, AA7050 or AA7010 or AA7040 (see U.S. Pat. No. 6,027,582) or AA7085 (see e.g. US Patent Application Publication No. 2002/0121319-A1) are used for these types of applications. Reduced quench sensitivity, that is deterioration of properties through thickness with lower quenching speed or thicker products, is a major wish from the aircraft manufacturers. Especially the properties in the ST-direction are a 15 major concern of the designers and manufacturers of structural parts.

20 For thick sections having a thickness of more than 3 inch or parts machined from such thick sections, a uniform and reliable property balance through thickness is important. Currently, AA7050 or AA7010 or AA7040 (see U.S. Pat. No. 6,027,582) or AA7085 (see e.g. US Patent Application Publication No. 2002/0121319-A1) are used for these types of applications. Reduced quench sensitivity, that is deterioration of properties through thickness with lower quenching speed or thicker products, is a major wish from the aircraft manufacturers. Especially the properties in the ST-direction are a 25 major concern of the designers and manufacturers of structural parts.

20 For thick sections having a thickness of more than 3 inch or parts machined from such thick sections, a uniform and reliable property balance through thickness is important. Currently, AA7050 or AA7010 or AA7040 (see U.S. Pat. No. 6,027,582) or AA7085 (see e.g. US Patent Application Publication No. 2002/0121319-A1) are used for these types of applications. Reduced quench sensitivity, that is deterioration of properties through thickness with lower quenching speed or thicker products, is a major wish from the aircraft manufacturers. Especially the properties in the ST-direction are a 30 major concern of the designers and manufacturers of structural parts.

30 A better performance of the aircraft, i.e. reduced manufacturing cost and reduced operation cost, can be achieved by improving the property balance of the aluminum alloys used in the structural part and preferably using only one type of alloy to reduce the cost of the alloy and to reduce the cost in the recycling of aluminum scrap and waste.

35 Accordingly, it is believed that there is a demand for an aluminum alloy capable of achieving the improved proper 40 property balance in almost every relevant product form.

**DESCRIPTION OF THE INVENTION**

It is an object of the present invention to provide AA2000-45 series alloys having improved property balance.

It is another object of the present invention to provide a 50 wrought aluminum alloy product of an AA2000-series alloy comprising 2 to 5.5% Cu, 0.5 to 2% Mg, at most 1% Mn, Fe <0.25%, Si >0.10 to 0.35%, having improved properties, in particular having improved fracture toughness.

It is another object of the present invention to provide an 55 AA2x24-series alloy having an improved property balance.

It is another object of the present invention to provide a 60 method of manufacturing such AA2000-series alloy products.

These and other objects and further advantages are met or 65 exceeded by the present invention method of manufacturing a wrought aluminum alloy product of an AA2000-series alloy, the method comprising the steps of:

- 60 a. casting stock of an ingot of an AA2000-series aluminum alloy comprising 2 to 5.5% Cu, 0.5 to 2% Mg, at most 1% Mn, Fe <0.25%, Si >0.10 to 0.35%,
- b. preheating and/or homogenizing the cast stock;
- c. hot working the stock by one or more methods selected from the group consisting of rolling, extrusion, and forging;
- d. optionally cold working the hot worked stock;

- e. solution heat treating (SHT) of the hot worked and optionally cold worked stock at a temperature and time sufficient to place into solid solution the soluble constituents in the aluminum alloy;
- f. cooling the SHT stock, preferably by one of spray quenching or immersion quenching in water or other quenching media;
- g. optionally stretching or compressing the cooled SHT stock or otherwise cold working the cooled SHT stock to relieve stresses, for example levelling or drawing or cold rolling of the cooled SHT stock;
- h. ageing of the cooled and optionally stretched or compressed or otherwise cold worked SHT stock to achieve a desired temper.

According to this invention there is at least one heat treatment carried out at a temperature in a range of more than 505° C. but lower than the solidus temperature of the subject aluminum alloy, and wherein this heat treatment is carried out either: (i) after the homogenisation heat treatment but prior to hot working, or (ii) after the solution heat treatment of step e), or (iii) both after the homogenisation heat treatment but prior to hot working and also after the solution heat treatment of step e).

The aluminum alloy can be provided as an ingot or slab or billet for fabrication into a suitable wrought product by casting techniques regular in the art for cast products, e.g. DC-casting, EMC-casting, EMS-casting. Slabs resulting from continuous casting, e.g. belt casters or roll casters, also may be used, which in particular may be advantageous when producing thinner gauge end products. Grain refiners such as those containing titanium and boron, or titanium and carbon, may also be used as is well-known in the art. After casting the alloy stock, the ingot is commonly scalped to remove segregation zones near the cast surface of the ingot.

It is known in the art that the purpose of a homogenisation heat treatment has the following objectives: (i) to dissolve as much as possible coarse soluble phases formed during solidification, and (ii) to reduce concentration gradients to facilitate the dissolution step. A preheat treatment achieves also some of these objectives. A typical preheat treatment for AA2×24-series alloys would be a temperature of 420 to 500° C. with a soaking time in the range of 3 to 50 hours, more typically for 3 to 20 hours.

Firstly, the soluble eutectic phases such as the S-phase in the alloy stock are dissolved using regular industry practice. This is typically carried out by heating the stock to a temperature of less than 500° C. as the S-phase eutectic phase ( $Al_2MgCu$ -phase) has a melting temperature of about 507° C. in AA2×24-series alloys. In AA2×24-series alloys there is also a  $\Theta$ -phase having a melting point of about 510° C. As is known in the art this can be achieved by a homogenisation treatment in said temperature range and allowing the stock to cool to the hot working temperature, or after homogenisation the stock is subsequently cooled and reheated to hot working temperature. The regular homogenisation process can also be done in two or more steps if desired, and which are typically carried out in a temperature range of 430 to 500° C. for AA2×24-series alloys. For example in a two step process, there is a first step between 457 and 463° C., and a second step between 470 and 493° C., to optimise the dissolving process of the various phases depending on the exact alloy composition.

The soaking time at the homogenisation temperature according to industry practice is alloy dependent as is well known to the skilled person, and is commonly in the range of about 1 to 50 hours. The heat-up rates that can be applied are those which are regular in the art.

This is where the homogenisation practice according to the prior art stops. However, it is an important aspect of the present invention that after the regular homogenisation practice where the alloy composition allows complete dissolution of soluble phases (eutectics) present from solidification at least one further heat treatment can be carried out at a temperature in a range of more than 500° C. but at a temperature lower than the solidus temperature of the subject alloy.

For the AA2000-series alloys processed according to the invention the preferred temperature is in a range of >505 to 550° C., preferably 505 to 540° C., and more preferably 510 to 535° C., and furthermore preferably at least 515° C.

For the system the soaking time at this further heat treatment is from about 1 to up about 50 hours. A more practical soaking time would not be more than about 30 hours, and preferably not more than about 15 hours. A too long soaking time at too high a temperature may lead to an undesired coarsening of dispersoids adversely affecting the mechanical properties of the final alloy product.

The skilled person will immediately recognise that at least the following alternative homogenisation practices can be used, while achieving the same technical effect:

- (a) regular homogenisation according to industry practice, wherein afterwards the temperature is further raised to carry out the additional step according to this invention, followed by cooling to hot working temperature, such as, for example, 470° C.
- (b) as alternative (a), but wherein after the additional step according to this invention the stock is cooled, for example to ambient temperature, and subsequently reheated to hot working temperature.
- (c) as alternative (a), but wherein between the heat treatment according to regular industry practice and the further heat treatment according to this invention the stock is being cooled, for example to below 150° C. or to ambient temperature,
- (d) a practice wherein between the various steps (regular practice, heat treatment according to invention, and heating to hot working temperature) the stock is cooled, for example to below 150° C. or to ambient temperature, where after it is reheated to the relevant temperature.

In the alternatives wherein following the heat treatment according to this invention the stock is firstly cooled to, for example, ambient temperature prior to reheating for hot working, preferably a fast cooling rate is used to prevent or at least minimise uncontrolled precipitation of various secondary phases, e.g.  $Al_2CuMg$  or  $Al_2Cu$ .

Following the preheat and/or homogenisation practice according to this invention the stock can be hot worked by one or more methods selected from the group consisting of rolling, extrusion, and forging, preferably using regular industry practice. The method of hot rolling is preferred for the present invention.

The hot working, and hot rolling in particular, may be performed to a final gauge, e.g. 3 mm or less or alternatively thick gauge products. Alternatively, the hot working step can be performed to provide stock at intermediate gauge, typical sheet or thin plate. Thereafter, this stock at intermediate gauge can be cold worked, e.g. by means of rolling, to a final gauge. Depending on the alloy composition and the amount of cold work an intermediate anneal may be used before or during the cold working operation.

In an embodiment of the method according to this invention following the regular practice of SHT and fast cooling for the subject aluminum alloy product, the stock is subjected to the further heat treatment according to this invention, one may designate this as a second SHT, at a higher temperature

than the first regular SHT, wherein afterwards the stock is rapidly cooled to avoid undesirable precipitation out of various phases. Between the first and second SHT the stock can be rapidly cooled according to regular practice, or alternatively the stock is ramped up in temperature from the first to the second SHT and after a sufficient soaking time it is subsequently rapidly cooled. This second SHT is to further enhance the properties in the alloy products and is preferably carried out in the same temperature range and time range as the homogenisation treatment according to this invention as set out in this description, together with the preferred narrower ranges. However, it is believed that also shorter soaking times can still be very useful, for example in the range of about 2 to 180 minutes. This further heat treatment may dissolve as much as practically possible any of the  $Mg_2Si$  phases which may have precipitated out during cooling for the homogenisation treatment or the during a hot working operation or any other intermediate thermal treatment. The solution heat treatment is typically carried out in a batch furnace, but can also be carried out in a continuous fashion. After solution heat treatment, it is important that the aluminum alloy be cooled to a temperature of 175° C. or lower, preferably to ambient temperature, to prevent or minimise the uncontrolled precipitation of secondary phases, e.g.  $Al_2CuMg$  and  $Al_2Cu$ . On the other hand cooling rates should preferably not be too high in order to allow for a sufficient flatness and low level of residual stresses in the product. Suitable cooling rates can be achieved with the use of water, e.g. water immersion or water jets.

Yet, in a further embodiment of this invention the defined AA2000-series alloy products are processed using regular homogenisation and/or preheat practice, and wherein afterwards the products are processed using the preferred SHT as set out above, thus regular SHT followed by the second solution heat treatment in the defined temperature and time range, together with the preferred narrower ranges. This will result in the same advantages in product properties. It is possible to carry out the first regular SHT followed by rapid cooling and reheating to the soaking temperature of the second SHT, alternatively the temperature is ramped up from the first to the second SHT and after a sufficient soaking time it is subsequently rapidly cooled.

The stock may be further cold worked, for example, by stretching in the range of about 0.5 to 10% of its original length to relieve residual stresses therein and to improve the flatness of the product. Preferably the stretching is in the range of about 0.5 to 6%, more preferably of about 0.5 to 5%. The stock can for example also be cold rolled with a rolling degree of for example 8 to 13%.

After cooling the stock is aged, typically at ambient temperatures, and/or alternatively the stock can be artificially aged. The artificial ageing can be of particular use for higher gauge products. Depending on the alloy system this ageing can be done by natural ageing, typically at ambient temperatures, or alternatively by means of artificially ageing. All ageing practices known in the art and those which may be subsequently developed can be applied to the AA2000-series alloy products obtained by the method according to this invention to develop the required strength and other engineering properties. Typical tempers would be for example T4, T3, T351, T39, T6, T651, T8, T851, and T89.

A desired structural shape is then machined from these heat treated plate sections, more often generally after artificial ageing, for example, an integral wing spar. SHT, quench, optional stress relief operations and artificial ageing are also followed in the manufacture of thick sections made by extrusion and/or forged processing steps.

The effect of the heat treatment according to this invention is that the damage tolerance properties are improved of the alloy product compared to the same aluminum alloy having also high Si content but processed without this practice according to the present invention. In particular an improvement can be found in one or more of the following properties: the fracture toughness, the fracture toughness in S-L orientation, the fracture toughness in S-T orientation, the elongation at fracture, the elongation at fracture in ST orientation, the fatigue properties, in particular FCGR, S—N fatigue or axial fatigue, the corrosion resistance, in particular exfoliation corrosion resistance, or SCC or IGC. It has been shown that there is a significant enhancement in mechanical properties of as much as 15%.

In addition, similar enhanced properties are achieved, or at least not adversely affected, with the aluminum alloy products according to this invention compared to the same alloy composition but having the regular low Si content and processed according to regular industry practice. This would allow the manufacturing of aluminum alloy product having similar or equivalent properties compared to the low Si alloys, but in a more cost effective manner as source material having a low Si-content is more expensive.

The following explanation for the surprisingly improved properties of the wrought product of this invention is put forward, with the caveat that it is merely an expression of belief and does not presently have complete experimental support.

The prior art refers to the  $Mg_2Si$  constituent phase as being insoluble in AA2000-series aluminum alloys and these particles are known fatigue initiation sites. In particular for aerospace applications, the prior art indicates that the Fe and Si content need to be controlled to very low levels to provide products with improved damage tolerant properties such as Fatigue Crack Growth Rate resistance (“FCGR”) and fracture toughness. From various prior art documents it is clear that the Si content is treated as an impurity and should be kept at a level as low as reasonably possible. For example US-2002/0121319-A1, incorporated herein by reference, discusses for an AA7000-series alloy the impact of these impurities on the alloying additions and states that Si will tie up some Mg thereby leaving an “Effective Mg” content available for solution, it is suggested that this be remedied by additional additions of Mg to compensate for the Mg tied up with the  $Mg_2Si$ , see section [0030] of US-2002/0121319-A1. However, at no point is it suggested that the  $Mg_2Si$  could be reintroduced into solution by a controlled heat treatment practice. With regard to the homogenisation practice it is mentioned that homogenisation may be conducted in a number of controlled steps but ultimately state that a preferred combined total volume fraction of soluble and insoluble constituents be kept low, preferably below 1% volume, see section [0102] of US-2002/0121319-A1. Within the examples, times and temperatures of heat treatments are given but at no point are the temperatures or times disclosed adequate in attempting the dissolution of  $Mg_2Si$  constituent particles, i.e. homogenisation temperature of up to 900° F. (482° C.) and solution treatment temperature of up to 900° F. (482° C.).

Also, for example U.S. Pat. No. 6,444,058, incorporated herein by reference, discusses for an AA2x24-series alloy that in order to improve on plane strain and plane stress toughness, fatigue resistance, or fatigue crack growth resistance that the second phase particles derived from Fe and Si and those derived from Cu and/or Mg are substantially eliminated by composition control and heat treatment. To that effect the Si content should be no greater than 0.05%, and the

heat treating temperature should be controlled at as high a temperature as possible while still being safely below the lowest incipient melting temperature of the alloy, which is about 935° F. (502° C.), see e.g. column 2, lines 35 to 52.

However, it has been found in accordance with the invention that for various AA2000-series aluminum alloys, the generally perceived constituent phase  $Mg_2Si$  is soluble via carefully controlled heat treatment and if they cannot be taken in complete solution then their morphology can be spherodised in such a way that fatigue and/or fracture toughness properties are improved. Once in solid solution, most of the Si and/or Mg will be available for subsequent ageing that may further enhance mechanical and corrosion properties. By deliberately increasing the Si content in the alloys according to this invention more of this Si is available for subsequent ageing practices but without having the detrimental coarse  $Mg_2Si$  phases in the final product. The gained improvements by the purposive addition of Si could also be sacrificed to some extent by making the alloy composition leaner in Mg and/or Cu thus improving the toughness of the alloy product. Thus the generally perceived detrimental impurity element Si is now being converted into a purposive alloying element having various advantageous technical effects.

For the AA2000-series alloys the upper limit for the Si content is about 0.35%, and preferably of about 0.25%, as a too high Si content may result in the formation of too coarse  $Mg_2Si$  phases which cannot be taken in complete solid solution and thereby adversely affecting the property improvements gained. The lower limit for the Si-content is >0.10%. A more preferred lower limit for the Si-content is about 0.15%, and more preferably about 0.17%.

A wrought AA2000-series aluminum alloy that can be processes favorably according to this invention, comprises, in wt. %:

Cu about 2 to 5.5%

Mg about 0.5 to 2%

Mn at most 1%

Zn <1.3%

Fe <0.25%, preferably <0.15%

Si >0.10 to 0.35%, preferably >0.10 to 0.25%, more preferably about 0.15 to 0.25%,

and optionally one or more elements selected from the group consisting of:

|    |                                              |
|----|----------------------------------------------|
| Zr | about 0.02 to 0.4%, preferably 0.04 to 0.25% |
| Ti | about 0.01 to 0.2%                           |
| V  | about 0.01 to 0.5%                           |
| Hf | about 0.01 to 0.4%                           |
| Cr | about 0.01 to 0.25%                          |
| Ag | at most 1%                                   |
| Sc | about 0.01 to 0.5%,                          |

balance being Al, incidental elements and impurities. Typically such impurities are present each <0.05%, total <0.15%.

Compared with the prior art, the alloy according to this invention has a high silicon content in the alloy composition, wherein the Si content is more than 0.10% and having a maximum of 0.35%. The rise in Si content has amongst others the advantage of improving the castability of the alloy.

In an embodiment of the AA2000-series alloy processed according to the invention the Cu content has a preferred lower limit of about 3.6%, and more preferably of about 3.8%. A preferred upper limit is of about 4.5%, and more preferably of 4%.

In an embodiment of the AA2000-series alloy processed according to the invention the Mg content has a preferred upper limit of 1.5%. In a more preferred embodiment the Mg is in a range of 1.1 to 1.3%.

The Mn content in the alloy according to the invention is preferably in a range of 0.1 to 0.9%, and more preferably in a range of 0.2 to 0.8%.

In an embodiment of the AA2000-series alloy processed according to this invention the Zn is present as an impurity element which can be tolerated to a level of at most about 0.3%, and preferably at most about 0.20%.

In another embodiment of the AA2000-series alloy processed according to this invention the Zn is purposively added to improve the damage tolerance properties of the alloy product. In this embodiment the Zn is typically present in a range of about 0.3 to 1.3%, and more preferably in a range of 0.45 to 1.1%.

If added, the Ag addition should not exceed 1.0%, and a preferred lower limit is 0.05%, more preferably about 0.1%. A preferred range for the Ag addition is about 0.20-0.8%. A more suitable range for the Ag addition is in the range of about 0.20 to 0.60%, and more preferably of about 0.25 to 0.50%, and most preferably in a range of about 0.3 to 0.48%.

In the embodiment where Ag it is not purposively added it is preferably kept at a low level of preferably <0.02%, more preferably <0.01%.

Zr can be added as dispersoid forming element, and is preferably added in a range of 0.02 to 0.4%, and more preferably in a range of 0.04 to 0.25%.

In another preferred embodiment of the invention the alloy has no deliberate addition of Cr and Zr as dispersoid forming elements. In practical terms this would mean that each of the Cr and Zr are at regular impurity levels of <0.05%, and preferably <0.03%, and more preferably the alloy is essentially free or substantially free from Cr and Zr. With "substantially free" and "essentially free" we mean that no purposeful addition of this alloying element was made to the composition, but that due to impurities and/or leaching from contact with manufacturing equipment, trace quantities of this element may, nevertheless, find their way into the final alloy product. In particular for thicker gauge products (e.g. more than 3 mm) the Cr ties up some of the Mg to form  $Al_{12}Mg_2Cr$  particles which adversely affect quench sensitivity of the wrought alloy product, and may form coarse particles at the grain boundaries thereby adversely affecting the damage tolerance properties. As dispersoid forming element it has been found that Zr is not as potent as Mn is in AA2x24-type aluminum alloys.

The Fe content for the alloy should be less than 0.25%. When the alloy product processed according to the invention is used for aerospace application preferably the lower-end of this range is preferred, e.g. less than about 0.10%, and more preferably less than about 0.08% to maintain in particular the toughness at a sufficiently high level. Where the alloy product is used for tooling plate application, a higher Fe content can be tolerated. However, it is believed that also for aerospace application a moderate Fe content, for example about 0.09 to 0.13%, or even about 0.10 to 0.15%, can be used. Although the skilled person would believe that this has an adverse effect on the toughness of the product, some of this loss in properties, if not all, is gained back when using the method according to this invention. The resultant would be an alloy product, although having moderate Fe levels, but when processed according to this invention it has properties equivalent to the same alloy product safe to a lower Fe content, e.g. 0.05 or 0.07%, when processed using regular practice. Thus similar properties are achieved at higher Fe-levels, which has a significant cost advantage as source material having very low Fe-contents is expensive.

In another preferred embodiment of the invention the AA2000-series alloy that can be processed favorably according to this invention has a composition, consisting of, in wt. %:

|    |                                                                                 |
|----|---------------------------------------------------------------------------------|
| Cu | 3.6 to 4.4, preferably 3.8 to 4.4                                               |
| Mg | 1.2 to 1.8                                                                      |
| Mn | 0.3 to 0.8                                                                      |
| Cr | max. 0.10, preferably max. 0.05                                                 |
| Zr | max. 0.05, preferably max. 0.03                                                 |
| Zn | max. 0.25                                                                       |
| Fe | max. 0.12, preferably max. 0.08                                                 |
| Si | >0.10 to 0.35, and preferably >0.10 to 0.25,<br>max. 0.15, preferably max. 0.10 |

balance aluminum and incidental elements and impurities. Typically such impurities are present each <0.05%, total <0.15%. This alloy composition embraces the AA2324 alloy (registered in 1978).

In another preferred embodiment of the invention the AA2000-series alloy that can be processed favourably according to this invention has a composition consisting of the AA2524 alloy (registered in 1995), but with the proviso that the Si is in the range of >0.10 to 0.35%, or an above-described preferred narrower range of the present invention. The composition ranges for the AA2524 alloy is, in wt. %:

|    |            |
|----|------------|
| Cu | 4.0-4.5    |
| Mn | 0.45-0.7   |
| Mg | 1.2-1.6    |
| Cr | max. 0.05  |
| Zn | max. 0.15  |
| Ti | max. 0.1   |
| Si | max. 0.06  |
| Fe | max. 0.12, |

incidental elements and impurities each <0.05, total <0.15, balance aluminum.

The AA2000-series alloy products manufactured according to this invention may be provided with a cladding. Such clad products utilise a core of the aluminum base alloy of the invention and a cladding of usually higher purity which in particular corrosion protects the core. The cladding includes, but is not limited to, essentially unalloyed aluminum or aluminum containing not more than 0.1 or 1% of all other elements. Aluminum alloys herein designated AA1xxx-type series include all Aluminum Association (AA) alloys, including the sub-classes of the 1000-type, 1100-type, 1200-type and 1300-type. Thus, the cladding on the core may be selected from various Aluminum Association alloys such as 1060, 1045, 1050, 1100, 1200, 1230, 1135, 1235, 1435, 1145, 1345, 1250, 1350, 1170, 1175, 1180, 1185, 1285, 1188, or 1199. In addition, alloys of the AA7000-series alloys, such as 7072 containing zinc (0.8 to 1.3%) or having about 0.3 to 0.7% Zn, can serve as the cladding and alloys of the AA6000-series alloys, such as 6003 or 6253, which contain typically more than 1% of alloying additions, can serve as cladding. Other alloys could also be useful as cladding as long as they provide in particular sufficient overall corrosion protection to the core alloy. The clad layer or layers are usually much thinner than the core, each constituting about 1 to 15 or 20 or possibly about 25% of the total composite thickness. A cladding layer more typically constitutes around 1 to 12% of the total composite thickness.

The AA2000-series alloy product processed according to this invention can be used amongst others in the thickness

range of at most 0.5 inch (12.5 mm), the properties will be excellent for fuselage sheet. In the thin plate thickness range of 0.7 to 3 inch (17.7 to 76 mm) the properties will be excellent for wing plate, e.g. lower wing plate. The thin plate thickness range can be used also for stringers or to form an integral wing panel and stringer for use in an aircraft wing structure. When processed to thicker gauges of more than 2.5 inch (63 mm) to about 11 inch (280 mm) excellent properties have been obtained for integral part machined from plates, or to form an integral spar for use in an aircraft wing structure, or in the form of a rib for use in an aircraft wing structure. The thicker gauge products can be used also as tooling plate, e.g. moulds for manufacturing formed plastic products, for example via die-casting or injection moulding. The alloy products processed according to the invention can also be provided in the form of a stepped extrusion or extruded spar for use in an aircraft structure, or in the form of a forged spar for use in an aircraft wing structure.

In the following, the invention will be explained by the following, non-limitative example.

#### Example

On a pilot scale of testing a billet have been DC-cast having a diameter of 250 mm and a length of over 850 mm. The alloy composition is listed in Table 1, and whereby it is noticed that alloy 3 has an Fe content slightly higher than what is currently customary for aerospace grade rolled products. Alloy 3 would be a typical example of the AA2324 series alloy, save to the higher Si and Fe contents. The alloy composition would also fall within the known compositional ranges of AA2524, save for the higher Si content. From the billet two rolling blocks have been machined having dimensions of 150×150×300 mm. By following this route blocks with an identical chemistry were obtained making it easier to fairly assess the influence of the heat treatments at a later stage on the properties. The blocks were all homogenised using the same cycles of 25 hours at 490° C. whereby industrial heat up rates and cooling rates were applied. Depending on the block a further homogenisation treatment according to the invention was applied whereby the furnace temperature is further increased and where after a second heat treatment or homogenisation treatment of 5 hours at 515° C. was applied. Following the homogenisation the blocks were cooled to room temperature. Thereafter all the blocks were preheated for 5 hours at 460° C. in one batch and hot rolled from 150 to 40 mm. The entrance temperatures (surface measurements) were in the range of 450 to 460° C. and mill exit temperatures varied in the range of 390 to 400° C. After hot rolling the plates received a one or two step solution heat treatment followed by a cold water quench. One further comparative sample (Sample 1A3) was processed using a more common SHT practice of 4 hours at 495° C. All the plates were naturally aged for 5 days to T4 temper. The plates were not stretched prior to ageing. All heat treatments are summarised in Table 2.

The average mechanical properties according to ASTM-B557 standard over 2 samples of the 40 mm plates produced with the various heat treatments are listed in Table 3 and wherein “TYS” stands for Tensile Yield Strength in MPa, UTS for Ultimate Tensile Strength in MPa, and “Kq” for the qualitative fracture toughness in MPa.v/m. The fracture toughness has been measured in accordance with ASTM B645. All testing was done at 1/2T.

## 11

TABLE 1

| Composition of the alloys, in wt. %, balance Al and regular impurities. |      |      |     |      |     |       |       |      |       |
|-------------------------------------------------------------------------|------|------|-----|------|-----|-------|-------|------|-------|
| Alloy                                                                   | Si   | Fe   | Cu  | Mn   | Mg  | Cr    | Zn    | Ti   | Zr    |
| 1                                                                       | 0.20 | 0.11 | 4.0 | 0.65 | 1.2 | <0.01 | <0.01 | 0.04 | <0.01 |

TABLE 2

| Sample | Homogenisation                    | Preheat       | SHT                             | Ageing |
|--------|-----------------------------------|---------------|---------------------------------|--------|
| 1A1    | 25 hrs@490° C.                    | 5 hrs@460° C. | 4 hrs@500° C.                   | T4     |
| 1A2    | 25 hrs@490° C.                    | 5 hrs@460° C. | 4 hrs@500° C. +<br>2 hr@515° C. | T4     |
| 1A3    | 25 hrs@490° C.                    | 5 hrs@460° C. | 4 hrs@495° C.                   | T4     |
| 1B1    | 25 hrs@490° C. +<br>5 hrs@515° C. | 5 hrs@460° C. | 4 hrs@500° C.                   | T4     |
| 1B2    | 25 hrs@490° C. +<br>5 hrs@515° C. | 5 hrs@460° C. | 4 hrs@500° C. +<br>2 hr@515° C. | T4     |

TABLE 3

| Sample | Mechanical properties of the various 40 mm plates. |     |     |     |     |     |     |     |     |  |
|--------|----------------------------------------------------|-----|-----|-----|-----|-----|-----|-----|-----|--|
|        | L                                                  |     | LT  |     | ST  |     | Kq  |     |     |  |
|        | TYS                                                | UTS | TYS | UTS | TYS | UTS | L-T | T-L | S-L |  |
| 1A1    | 320                                                | 500 | 302 | 472 | 302 | 441 | 54  | 44  | 33  |  |
| 1A2    | 324                                                | 505 | 304 | 475 | 302 | 459 | 52  | 46  | 37  |  |
| 1A3    | 318                                                | 492 | 298 | 464 | 296 | 446 | 49  | 41  | 32  |  |
| 1B1    | 311                                                | 486 | 298 | 468 | 297 | 436 | 55  | 47  | 33  |  |
| 1B2    | 320                                                | 501 | 306 | 480 | 306 | 442 | 52  | 48  | 34  |  |

TABLE 4

| Specific data taken from the prior art. |     |     |    |     |     |    |     |     |    |     |     |     |
|-----------------------------------------|-----|-----|----|-----|-----|----|-----|-----|----|-----|-----|-----|
| Ref.                                    | L   |     |    | LT  |     |    | ST  |     |    | Kq  |     |     |
|                                         | TYS | UTS | EI | TYS | UTS | EI | TYS | UTS | EI | L-T | T-L | S-L |
| A                                       | 310 | 430 | 10 | 300 | 420 | 8  | 260 | 380 | 4  | 45  | 40  | —   |

From the results of Table 3 with respect to the mechanical properties the following can be seen:

The plate produced via a standard processing (Sample 1A3) has generally the lowest set of properties. The other samples exhibit better properties when using higher processing temperatures, especially the toughness is improved with on average 10%. Further improvements, in particular in toughness, can be made by lowering the Fe content to standard aerospace levels of <0.05%.

The current set of obtained properties despite the high Si and relatively high Fe levels, and especially sample 1A2 and 1B2, meet the Airbus specification AIMS 03-02-020, Issue 3, February 2002, for 2024/2xxx T351 plate (incorporated herein by reference) even though the plates processed according to the invention have a relatively high Fe levels and are in T4 temper.

Having now fully described the invention, it will be apparent to one of ordinary skill in the art that many changes and modifications can be made without departing from the spirit or scope of the invention as herein described.

## 12

The invention claimed is:

1. A method of manufacturing a wrought aluminum alloy product of an AA2000-series alloy, the method comprising the steps of:
    - a. casting stock of an ingot of an AA2000-series aluminum alloy;
    - b. preheating and/or homogenising the cast stock at a temperature in a range of 430 to 500° C.;
    - c. heat treating the cast stock at a temperature in a range of more than 505° C. but lower than the solidus temperature of the subject aluminum alloy;
    - d. hot working the stock by one or more methods selected from the group consisting of rolling, extrusion, and forging;
    - e. optionally cold working the hot worked stock;
    - f. first solution heat treating (SHT) of the hot worked and optionally cold worked stock;
    - g. second solution heat treating of the worked stock at a higher temperature than the first SHT, the temperature being in a range of more than 505° C. but lower than the solidus temperature of the subject aluminium alloy and then rapidly cooling the SHT stock;
    - h. optionally stretching or compressing the SHT stock that has undergone the second solution heat treating and rapid cooling or otherwise cold working the SHT stock that has undergone the second solution heat treating and rapid cooling;
  - i. ageing of the cooled and optionally stretched or compressed or otherwise cold worked SHT stock to achieve a desired temper;
- wherein the heat treatment after the homogenisation heat treatment prior to hot working and the second solution heat treatment after the first solution heat treatment each has a soaking time of from about one to about 50 hours, and

wherein the AA2000-series aluminum alloy product has a composition within the range of an aluminum alloy product selected from the group consisting of AA2324 with the proviso that the Si content is in a range of >0.10 to 0.35%, such that the alloy composition consists of, in wt. %:

|    |               |
|----|---------------|
| Cu | 3.8-4.4       |
| Mn | 0.30-0.9      |
| Mg | 1.2-1.8       |
| Cr | max. 0.10     |
| Zn | max. 0.25     |
| Ti | max. 0.15     |
| Si | >0.10 to 0.35 |
| Fe | max. 0.12,    |

incidental elements and impurities, each <0.05, total <0.15, balance aluminium, and

## 13

AA2524 with the proviso that the Si content is in a range of >0.10 to 0.35%, such that the alloy composition consists of, in wt. %:

|    |               |
|----|---------------|
| Cu | 4.0-4.5       |
| Mn | 0.45-0.7      |
| Mg | 1.2-1.6       |
| Cr | max. 0.05     |
| Zn | max. 0.15     |
| Ti | max. 0.1      |
| Si | >0.10 to 0.35 |
| Fe | max. 0.12,    |

incidental elements and impurities each <0.05, total <0.15, balance aluminium.

2. Method according to claim 1, wherein the AA2000-series aluminum alloy has a Si-content in the range of >0.10 to 0.25%.

3. Method according to claim 1, wherein the AA2000-series aluminum alloy has a Si-content in the range of 0.15 to 0.25%.

4. Method according to claim 1, wherein the AA2000-series aluminum alloy has a Si-content is 0.17 to 0.35%.

5. Method according to claim 1, wherein the AA2000-series aluminum alloy has an Fe content of less than 0.10%.

6. Method according to claim 1, wherein the AA2000-series aluminum alloy has an Fe content of less than 0.08%.

7. Method according to claim 1, wherein the AA2000-series aluminum alloy has a Cr content of <0.05%.

8. Method according to claim 1, wherein the AA2000-series aluminum alloy has a Cr content of <0.03%.

9. Method according to claim 1, wherein at least one heat treatment is carried out at a temperature range of at least 515 to 550° C.

10. Method according to claim 1, wherein at least one heat treatment is carried out at a temperature range of at least 515 to 535° C.

11. Method according to claim 1, wherein the hot working is carried out by rolling.

12. Method according to claim 1, wherein the hot working is carried out by extrusion.

13. Method according to claim 1, wherein heat treating of step (c) and second solution heat treating of step (g) are carried out at a temperature in a range of at least 515° C. but lower than the solidus temperature of the subject aluminum alloy to dissolve constituent phase Mg<sub>2</sub>Si.

14. Method according to claim 1, wherein the AA2000-series aluminum alloy product has a gauge of at least 3 mm.

15. Method according to claim 1, wherein the AA2000-series aluminum alloy product has a gauge of at least 30 mm.

16. Method according to claim 1, wherein the AA2000-series aluminum alloy product has a gauge in a range of 30 to 300 mm.

17. Method according to claim 1, wherein the AA2000-series aluminum alloy product has the composition within the range of AA2324 with the proviso that the Si content is in a range of >0.10 to 0.35%, such that the alloy composition consists of, in wt. %:

|    |           |
|----|-----------|
| Cu | 3.8-4.4   |
| Mn | 0.30-0.9  |
| Mg | 1.2-1.8   |
| Cr | max. 0.10 |
| Zn | max. 0.25 |

## 14

-continued

|    |               |
|----|---------------|
| Ti | max. 0.15     |
| Si | >0.10 to 0.35 |
| Fe | max. 0.12,    |

5 incidental elements and impurities, each <0.05, total <0.15, balance aluminum.

18. Method according to claim 17, wherein the AA2000-series aluminum alloy product has Si content in a range of >0.10 to 0.25% and Cu content in a range of 3.8-4%.

19. Method according to claim 1, wherein the AA2000-series aluminum alloy product has the composition within the range of AA2524 with the proviso that the Si content is in a range of >0.10 to 0.35%, such that the alloy composition consists of, in wt. %:

|    |               |
|----|---------------|
| Cu | 4.0-4.5       |
| Mn | 0.45-0.7      |
| Mg | 1.2-1.6       |
| Cr | max. 0.05     |
| Zn | max. 0.15     |
| Ti | max. 0.1      |
| Si | >0.10 to 0.35 |
| Fe | max. 0.12,    |

25 incidental elements and impurities each <0.05, total <0.15, balance aluminum.

20. Method according to claim 1, wherein the AA2000-series aluminum alloy product is selected from the group comprising fuselage sheet, fuselage frame member, lower wing plate, thick plate for machined parts, thin sheet for stringers, spar member, and rib member.

21. Method according to claim 1, wherein the AA2000-series aluminum alloy product is in the form of a mold plate or a tooling plate.

22. The method of claim 1, wherein the second solution heat treating after said first solution heat treating occurs after rapidly cooling the first SHT stock and comprises reheating the cooled first SHT stock to a temperature of at least 515° C. but lower than the solidus temperature of the subject aluminum alloy as a soaking temperature of the second solution heat treating and wherein after the second solution heat treating the stock is rapidly cooled prior to said ageing.

23. The method of claim 22, wherein each said rapid cooling cools the stock to a temperature of 175° C. or lower.

24. The method according to claim 1, wherein the second solution heat treatment has a soaking time of about 2 hours.

25. The method according to claim 1, wherein the heat treatment after the homogenisation has a soaking time of about 5 hours and the second solution heat treatment has a soaking time of about 2 hours.

26. The method of claim 1, wherein the second solution heat treating has a soaking time of from about 2 to about 15 hours, wherein the soaking temperature of the first solution heat treating is in the range from 495-500° C.; wherein the AA2000-series aluminum alloy product has the composition consisting of, in wt. %:

|    |          |
|----|----------|
| Cu | 3.8-4    |
| Mn | 0.65-0.9 |
| Mg | 1.2-1.5  |
| Cr | <0.10    |
| Zn | <0.25    |

|    |               |
|----|---------------|
| Ti | max. 0.15     |
| Si | >0.10 to 0.25 |

|                                                       |                          |
|-------------------------------------------------------|--------------------------|
| Fe                                                    | max. 0.12,               |
| incidental elements and impurities, each <0.05, total | <0.15, balance aluminum. |

## 15

27. A method of manufacturing a wrought aluminum alloy product of an AA2000-series alloy, the method comprising the steps of:

a. casting stock of an ingot of an AA2000-series aluminum alloy having a chemical composition comprising, in wt. %:

Cu content of 2 to 4%,

Mg 0.5 to 2%,

Mn at most 1%

Zn <1.3%

Fe <0.25%

Si >0.10 to 0.35%,

balance being Al, incidental elements and impurities;

b. preheating and/or homogenising the cast stock at a temperature in a range of 430 to 500° C.;

c. heat treating the cast stock at a temperature in a range of more than 505° C. but lower than the solidus temperature of the subject aluminum alloy;

d. hot working the stock by one or more methods selected from the group consisting of rolling, extrusion, and forging;

e. optionally cold working the hot worked stock;

f. first solution heat treating (SHT) of the hot worked and optionally cold worked stock;

g. second solution heat treating of the worked stock at a higher temperature than the first SHT, the temperature being in a range of more than 505° C. but lower than the solidus temperature of the subject aluminium alloy and then rapidly cooling the SHT stock;

h. optionally stretching or compressing the SHT stock that has undergone the second solution heat treating and rapid cooling or otherwise cold working the SHT stock that has undergone the second solution heat treating and rapid cooling to relieve stresses by at least one cold working step selected from the group consisting of levelling or drawing or cold rolling of the SHT stock that has undergone the second solution heat treating and rapid cooling;

i. ageing of the cooled and optionally stretched or compressed or otherwise cold worked SHT stock to achieve a desired temper;

and wherein the heat treatment after the homogenisation heat treatment prior to hot working and the second

## 16

solution heat treatment after the first solution heat treatment each has a soaking time of from about one to about 50 hours.

28. Method according to claim 27, wherein the AA2000-series aluminum alloy further comprises one or more elements, in wt. %, selected from the group consisting of:

|    |    |               |
|----|----|---------------|
| 10 | Zr | 0.02 to 0.4%  |
|    | Ti | 0.01 to 0.2%  |
|    | V  | 0.01 to 0.5%  |
|    | Hf | 0.01 to 0.4%  |
|    | Cr | 0.01 to 0.25% |
|    | Ag | at most 1%,   |
|    | Sc | 0.01 to 0.5%. |

29. Method according to claim 27, wherein the AA2000-series aluminum alloy has an Fe content of less than 0.15%.

30. Method according to claim 27, wherein the AA2000-series aluminum alloy further comprises a Zr content of <0.05%.

31. Method according to claim 27, wherein the AA2000-series aluminum alloy further comprises a Zr content of <0.03%.

32. Method according to claim 27, wherein the AA2000-series aluminum alloy has a Mg content of 0.5 to 1.5%.

33. Method according to claim 27, wherein the AA2000-series aluminum alloy has a Zn content of at most 0.3%.

34. Method according to claim 27, wherein the AA2000-series aluminum alloy has a Mn content of in a range of 0.1 to 0.9%.

35. The method of claim 27, wherein the AA2000-series aluminum alloy product has a gauge of at least 30 mm.

36. The method of claim 27, wherein the second solution heat treating after said first solution heat treating occurs after rapidly cooling the first SHT stock and comprises reheating the cooled first SHT stock to a temperature of at least 515° C. but lower than the solidus temperature of the subject aluminium alloy as a soaking temperature of the second solution heat treating, and wherein after the second solution heat treating the stock is rapidly cooled prior to said ageing.

37. The method of claim 36, wherein each said rapid cooling cools the stock to a temperature of 175° C. or lower.

\* \* \* \* \*